

## UNITED STATES PATENT OFFICE

2,615,805

## MANUFACTURE OF LEAD

Leonard F. Taylor, South Darley, near Matlock, and Patrick W. Wright, Holloway, near Matlock, England, assignors to H. J. Enthoven & Sons Limited, London, England, a British company

No Drawing. Application April 17, 1950, Serial No. 156,488. In Great Britain May 11, 1948

## 1 Claim. (Cl. 75—166)

1

This invention relates to the manufacture of lead. In the industrial employment of lead for pipes and vessel linings and the like the degree of purity of the lead is important in many cases, for example, when the lead is used in chemical plants. On the other hand, lead as manufactured is very liable to contain impurities such as antimony, silver, bismuth, arsenic, tin and copper.

One of the tests laid down by the British Standards Institution in their British Standard Specification (B. S. S. No. 334 of 1934) for chemical lead is the so-called "flash-test" which depends on the peculiar behaviour of a sample of lead at a particular temperature (the flash-point) when immersed in concentrated sulphuric acid and heated.

An investigation by us into the effect of various percentages of different impurities upon the flash-point of lead has revealed some very interesting facts. In particular it has been ascertained that quite small amounts of some metal impurities in lead lower the flash-point considerably, this being particularly the case with antimony. For example, whereas the flash-point of a sample of lead substantially free from antimony was 322° C., the flash-point of lead containing 0.01% of antimony was 248° C., containing 0.02% antimony was 243° C., containing 0.03% antimony 240° C., and containing 0.04% antimony 238° C.

We have found, much to our surprise, that the presence of a small amount of nickel in lead of progressively increased antimony content—which lead normally suffers from a sharp and progressive drop in flash-point as above noted—has its flash-point actually raised. For example 0.01 per cent of nickel in addition to from 0.01 to 0.02 per cent of antimony raises the flash-point to about 326° C. Similarly 0.02 per cent of nickel in addition to from 0.01 to 0.03 per cent of antimony raises the flash-point to 330° C.

The present invention, therefore, consists in partially or completely eliminating the adverse effect of antimony in lowering the flash-point of lead, or even raising the flash-point of lead, notwithstanding the presence of a small amount of antimony by incorporating therein a small amount of nickel. From the industrial standpoint the importance of being able to maintain

2

and even raise the flash-point of lead without resorting to the expense of extreme refining is apparent, and from this point of view the invention consists in deliberately desisting from refining lead as regards antimony content beyond about 0.03 per cent and by adding a small per cent of nickel to compensate for the antimony content.

The greater the amount of nickel introduced 10 the greater may be the amount of antimony left in the lead, as is indicated by the following table of contents and flash-points:

[Flash-points, ° C.]

| Antimony content of lead.....percent.. | Nil  | 0.01 | 0.02 | 0.03 | 0.04 | 0.05 | 0.06  |
|----------------------------------------|------|------|------|------|------|------|-------|
| Lead antimony only.....                | ° C. | ° C. | ° C. | ° C. | ° C. | ° C. | ° C.  |
| 322                                    | 248  | 243  | 240  | 238  | 238  | 238  | 238   |
| Lead antimony.....0.01% Ni.....        | 321  | 326  | 326  | 319  | 314  | 311  | 309   |
| Lead antimony.....0.02% Ni.....        | 321  | 330  | 330  | 330  | 328  | 326  | 323   |
| Lead antimony.....0.028% Ni.....       | 322  | 329  | 330  | 330  | 330  | 330  | ----- |

## 25 What we claim is:

Lead containing from 0.01 to 0.06 per cent by weight of antimony together with nickel ranging from 0.01 to 0.03 per cent by weight, the remainder being lead, the nickel serving to obviate the adverse effect of the antimony in lowering the flash-point of the lead.

L. F. TAYLOR.  
P. W. WRIGHT.

## 35 REFERENCES CITED

The following references are of record in the file of this patent:

## UNITED STATES PATENTS

| Number    | Name          | Date          |
|-----------|---------------|---------------|
| 2,067,507 | Smith -----   | Jan. 12, 1937 |
| 2,115,300 | Butcher ----- | Apr. 26, 1938 |

## FOREIGN PATENTS

| Number  | Country             | Date          |
|---------|---------------------|---------------|
| 326,818 | Great Britain ----- | Mar. 18, 1930 |

## 50 OTHER REFERENCES

The Metal Industry Handbook and Directory, 1948, page 151. Louis Cassier Co., London, England.